

## UNITED STATES PATENT OFFICE

ALBERT M. CLIFFORD, OF AKRON, OHIO, ASSIGNOR TO THE GOODYEAR TIRE & RUBBER COMPANY, OF AKRON, OHIO, A CORPORATION OF OHIO

## AGE RESISTER FOR RUBBER COMPOUNDS

No Drawing.

Application filed April 8, 1930. Serial No. 442,713.

My invention relates to methods of treating organic compounds and to the product formed thereby, and it has particular relation to methods of preserving such substances from premature deterioration. One of the objects of the invention is to provide a method of treating compounds of the above indicated class whereby to retard the deleterious effect of oxygen, heat, light and similar deteriorating agencies.

Heretofore, it has been observed that rubber, transformer oils, soaps and similar organic materials are attacked by, and gradually deteriorate under the influence of, atmospheric oxygen, sunlight, heat, etc. It has been proposed to overcome these deleterious effects by incorporating into the compounds certain preservatives known as anti-oxidants or age retarders. Although many materials have been employed for this purpose, the phenyl naphthylamines and similar secondary amines have been found by actual test to be among the most satisfactory for general use.

This invention consists in the discovery that aliphatic substituted phenyl naphthylamines such as cumidyl and xylyl naphthylamines, either of the alpha or beta form, are also excellent anti-oxidants which are practically equal in power as preservatives to the unsubstituted amines which have heretofore been employed. Substituted amines may be manufactured by methods analogous to those employed in the manufacture of phenyl naphthylamines merely by subjecting the naphthol (either alpha or beta) to a temperature of 280° to 310° C. in an autoclave for a period of eight to ten hours. The reaction products may be purified by washing them with dilute alkali in order to remove any unreacted naphthol and then following this treatment with subsequent washings with water, dilute acid, and finally with water. The product may be dried by subjecting it to distillation under vacuum. 1-3-4-xylyl beta naphthylamine

obtained in this manner is an orange colored oily material having a boiling point of 238° to 240° C at a pressure of seven millimeters of mercury. Cumidyl beta naphthylamine is also an orange colored material having a thick sirupy consistency and having a boiling point of 215° to 230° C. under a pressure of four millimeters of mercury. The compounds are both soluble in benzene, alcohol, acetic acid, etc., and are slightly soluble in petroleum ether. All of the solutions are characterized by deep blue fluorescence.

Although these materials may successfully be employed as antioxidants in most of the standard rubber compounds, the following is an example of a formula which has been found by actual test to be quite satisfactory:

|                          | Parts  |
|--------------------------|--------|
| Acetone extracted rubber | 100 65 |
| Zinc oxide               | 5      |
| Sulphur                  | 3      |
| Hexamethylene tetramine  | 1      |
| Stearic acid             | 1.5    |
| Antioxidant              | 1 70   |

Samples of compounds prepared in accordance with the preceding formula in which cumidyl beta naphthylamine and xylyl beta naphthylamine were employed as anti-oxidants were subjected to vulcanization for varying periods of time. One portion of these samples was then subjected immediately to physical tests in order to ascertain the tensile strength and elasticity thereof prior to aging.

A second set of exactly corresponding samples were then subjected to artificial aging in an oxygen bomb under pressure of 150 pounds per square inch and at a temperature of 50° C. for a period of six days. These samples were then removed from the bomb and subjected to physical tests identical with those conducted upon unaged samples.

The results of these tests are tabulated as follows:

| 5                                            | Cure | Tensile strength kgs/cm <sup>2</sup> | Per cent elong. | Load in kgs/cm <sup>2</sup> at |             | % weight increase |  |  |  |  |
|----------------------------------------------|------|--------------------------------------|-----------------|--------------------------------|-------------|-------------------|--|--|--|--|
|                                              |      |                                      |                 | 500% elong.                    | 700% elong. |                   |  |  |  |  |
| <i>Cumidyl beta naphthylamine</i>            |      |                                      |                 |                                |             |                   |  |  |  |  |
| 10      ORIGINAL                             |      |                                      |                 |                                |             |                   |  |  |  |  |
|                                              |      | 35                                   | 98              | 890                            | 14          | 45                |  |  |  |  |
|                                              |      | 50                                   | 146             | 860                            | 20          | 60                |  |  |  |  |
|                                              |      | 70                                   | 185             | 820                            | 26          | 92                |  |  |  |  |
| 15      AGED IN OXYGEN BOMB 6 DAYS AT 50° C. |      |                                      |                 |                                |             |                   |  |  |  |  |
|                                              |      | 35                                   | 104             | 835                            | 15          | 49                |  |  |  |  |
|                                              |      | 50                                   | 147             | 810                            | 23          | 80                |  |  |  |  |
|                                              |      | 70                                   | 167             | 780                            | 32          | 118               |  |  |  |  |
| 20 <i>Xylyl beta naphthylamine</i>           |      |                                      |                 |                                |             |                   |  |  |  |  |
| 25      ORIGINAL                             |      |                                      |                 |                                |             |                   |  |  |  |  |
|                                              |      | 35                                   | 112             | 905                            | 15          | 38                |  |  |  |  |
|                                              |      | 50                                   | 140             | 850                            | 20          | 58                |  |  |  |  |
|                                              |      | 70                                   | 172             | 810                            | 26          | 90                |  |  |  |  |
| 30      AGED IN OXYGEN BOMB 6 DAYS AT 50° C. |      |                                      |                 |                                |             |                   |  |  |  |  |
|                                              |      | 35                                   | 117             | 835                            | 17          | 56                |  |  |  |  |
|                                              |      | 50                                   | 137             | 785                            | 24          | 87                |  |  |  |  |
|                                              |      | 70                                   | 158             | 745                            | 33          | 122               |  |  |  |  |

It will be observed that the samples of material containing the new antioxidants are not materially affected by the action of oxygen even under the relatively severe conditions existing in the oxygen bomb. In fact, it would appear that the condition of the samples is somewhat improved, at least in certain cases, by such treatment. Under similar conditions, samples of material containing no antioxidants are reduced to resinous masses substantially devoid of elasticity and tensile strength.

The new antioxidants may be manufactured at relatively slight expense and trouble. They also possess but slight, if any, odor and are not appreciably toxic. They blend readily with rubber and also with other organic materials, such as transformer oils and soaps; in fact, the solubility thereof in organic materials appears to be somewhat greater than that of the simple phenyl naphthylamine compounds from which they may be considered as being derived. For these reasons, they are highly desirable as commercial materials.

Although I have described the preferred embodiments of the invention, it will be apparent to those skilled in the art that it is not limited thereto but that various modifications may be made therein without departing from the spirit of the invention or from the scope of the appended claims.

What I claim is:

1. A method of preserving rubber, transformer oils, soaps, and similar readily de-

composable organic materials which comprises incorporating therein a cumidyl naphthylamine.

2. A method of preserving rubber which comprises incorporating therein a cumidyl naphthylamine.

3. A rubber product that has been vulcanized in the presence of a cumidyl naphthylamine.

4. As a new chemical compound, a material having the formula



80

in which R is a cumidyl group.

In witness whereof, I have hereunto signed my name at Akron, in the county of Summit and State of Ohio, U. S. A., this 7th day of April, 1930.

ALBERT M. CLIFFORD.

85

90

95

100

105

110

115

120

125

130